

1

3,573,333

## LUBRICANT ADDITIVES FOR OXIDATION INHIBITION AND RUST INHIBITION

Jonathan L. Snead, Philadelphia, Joseph F. Messina, Havertown, and Henry Gisser, Philadelphia, Pa., assignors to the United States of America as represented by the Secretary of the Army

No Drawing. Continuation of application Ser. No. 613,077, Jan. 30, 1967. This application Aug. 19, 1969, Ser. No. 853,600

Int. Cl. C08h 17/36

U.S. CL. 260—413

1 Claim

### ABSTRACT OF THE DISCLOSURE

New compositions of matter are provided which are useful as additives in lubricants and which are oxidatively autoinhibitive and/or rust-inhibitive, the compositions comprising substituted phenylalkanes or hydroxyarylstearic acids or salts thereof wherein the aryl groups are attached to the alkyl chain at a tertiary carbon atom.

This application is a continuation of application Ser. No. 613,077, filed Jan. 30, 1967, now abandoned.

This invention relates to compounds useful as lubricant additives and more particularly concerns compounds which are oxidatively autoinhibitive and/or rust inhibitive.

Diesters and hydrocarbons are widely used as lubricants for such mechanisms as jet engines and hydraulic systems. These organic fluids are subject to oxidation, with consequent deterioration in physical and chemical properties. The addition of inhibitors is only a partial solution to the oxidation problem, in that the effects are short-lived unless sufficiently high concentrations are added, in which case, however, the other properties of the fluid, such as viscosity and liquid range, may be undesirably altered.

In the oxidation of hydrocarbons, for example, oxidation will occur preferentially at a tertiary C—H bond and the same is true of saturated aliphatic diesters. In general, the order of increasing resistance to oxidative attack a C—H bonds is tertiary, secondary, and primary. This is to be expected from the free radical nature of the oxidation process and the fact that the relative probability of attack of alkyl radicals at C—H bonds decreases in the order aforementioned.

These theoretical principles have been utilized in our invention to produce compounds that generate oxidation inhibitors. More specifically, selected aromatic groups have been attached to tertiary C—H bonds of hydrocarbons by synthesis. These compounds when subjected to oxidation, form hydroperoxides which break down to yield phenols, the active antioxidants. The phenols thus generated are capable of slowing down further oxidation of the remaining substrate (original compound) or other substrates which are less stable to oxidation.

Another aspect of the invention involves incorporating select groups on the tertiary C—H bond of long-chain fatty acids and fatty acid salts (soaps) to produce compounds which possess combined oxidation and rust inhibitory properties. The long hydrocarbon chain terminated by the strongly polar acid (or salt) group is an effective rust inhibitor. At the same time, the phenolic side chain, effective in preventing rapid oxidation, when oxidized, forms hydroperoxides that break down to yield other phenols more effective as antioxidants than the original compound.

It is therefore an object of this invention to provide improved lubricant additives which impart good oxidation stability to the lubricant.

2

Another object of the invention is to provide improved lubricant additives which impart good rust-inhibitive properties to the lubricant.

Still another object of the invention is to provide an additive to lubricant fluids which yields both good oxidation stability and good rust-inhibitive properties, said additive comprising but a single molecule.

Other and further objects of the invention will be apparent to those skilled in the art upon study of this disclosure.

Now in accordance with our present invention, the inhibitor-generating hydrocarbon above described will be an electron-donating, substituted phenylalkane where-in the ring is attached to the alkyl group at a tertiary carbon atom. The following compounds are examples of the type of structures involved:



When the compounds with the above molecular structures are added to oxidatively unstable compounds, the oxidation rates of the latter are decreased or completely inhibited, as illustrated by the data below:

TABLE I.—OXIDATION RATES OF MIXTURES OF SEC-BUTYLBENZENE AND INHIBITOR-GENERATING HYDROCARBONS AT 100° C.

| Inhibitor additive             | Mole, percent | Rate <sup>1</sup> | Time, hours |
|--------------------------------|---------------|-------------------|-------------|
| None                           | 0             | 7.2               | 5-10        |
| 4-sec-butyl-4'-methoxybiphenyl | 6.8           | 1.4               | 5-10        |
| 4-sec-butylbiphenyl            | 7.4           | 5.0               | 5-10        |

<sup>1</sup> Moles O<sub>2</sub>/mole compound per hour  $\times 10^4$ .

As an example, the inhibitor-generating compound 4-sec-butyl-4'-methoxybiphenyl may be prepared as follows:

p-Phenylanisole (46 g.; 0.25 mole) in 700 ml. of hot heptane was placed in a one-liter four-necked flask, fitted with a stirrer, reflux, dropping funnel, and a thermometer. Anhydrous AlCl<sub>3</sub> (13.3 g.; 0.1 mole) was added and the temperature maintained at 75–85° C. with the addition of chlorobutane (25 g.; 0.27 mole) over a period of 2.5 hours, with stirring. Stirring and heating at 75–85° C. was continued for 5.5 hours or until evolution of hydrogen chloride had ceased. The reaction mixture was poured over an equivalent amount (by volume) of crushed ice, with vigorous stirring, to hydrolyze the complex. The organic layer was washed free of acid with distilled water; dried over anhydrous Na<sub>2</sub>SO<sub>4</sub>; filtered, and the heptane removed under reduced pressure. The unreacted solid p-phenylanisole was distilled, in vacuo, using a steam-jacketed condenser. The residue was distilled in a pot still at 15–20 microns pressure. The liquid distillate was then fractionated through a short Vigreux column to yield 4-sec-butyl-4'-methoxybiphenyl, B.P. 137° C. at 0.65 mm.

Oxidation stability of the mixtures of unstable compounds and inhibitor additives was determined at 100° C. by using standard Warburg manometry as described by Umbreit, Burria, and Stauffer, "Manometric Techniques," pp. 1–17, 46–7, 77–8, Burgess Publishing Co., Minneapolis, Minn., 1959. One milliliter of compound was introduced into the main compartment of the Warburg flask. Since oxygen consumption in the initial stages of autoxidation was measured, it was not necessary to use absorbents for volatiles. The flask was immersed in a 100° C. oil

bath and allowed to come to equilibrium, during which time the system was flushed with oxygen for approximately 15 minutes. When the system was finally closed to the

until after the induction period and a considerable increase in acidity and viscosity was obtained. The results are presented in Table II below:

TABLE II.—OXIDATION OF ARYLSTEARIC ACIDS IN BIS(2-ETHYLHEXYL) SEBACATE<sup>1</sup>

| Additive                                                     | Neutralization number increase, <sup>2</sup> Eq. mg.<br>KOH/g. oil, hours |      |     |      |                       | Viscosity increase, <sup>3</sup> percent at<br>37.8° C., hours |      |      |      |    |     |     | Induction<br>period,<br>hours |      |
|--------------------------------------------------------------|---------------------------------------------------------------------------|------|-----|------|-----------------------|----------------------------------------------------------------|------|------|------|----|-----|-----|-------------------------------|------|
|                                                              | 24                                                                        | 48   | 72  | 96   | 240 at<br>168 150° C. | 336                                                            | 24   | 48   | 72   | 96 | 168 | 240 | 336                           |      |
| None                                                         | 23                                                                        |      |     |      |                       |                                                                | 75.0 |      |      |    |     |     |                               | 10   |
| 9(or 10)-(2-hydroxy-5-tert-butylphenyl)stearic acid          | 0.1                                                                       | 7.6  |     |      |                       |                                                                | 1.8  | 24   |      |    |     |     |                               | 37   |
| 9(or 10)-(2,3-dihydroxyphenyl)stearic acid                   | 0.2                                                                       | 0.2  | 6.8 |      |                       |                                                                | 1.1  | 1.7  | 21   |    |     |     |                               | 62   |
| 9(or 10)-(2-hydroxy-3-isopropyl-6-methyl-phenyl)stearic acid | 0.1                                                                       | 12   |     |      |                       |                                                                | 1.7  | 61   |      |    |     |     |                               | 38   |
| 9,12-Bis(4-hydroxyphenyl)stearic acid                        | 0.2                                                                       | 0.3  | 0.1 | —    | —0.5                  | —0.4                                                           | 0.7  | 2.5  | 1.7  | —  | 1.8 | 0   |                               | >240 |
| Calcium 9(or 10)-p-hydroxyphenyl stearate                    | 0                                                                         | 0    | 7.7 |      |                       |                                                                | 1.6  | —2.4 | 17.7 |    |     |     |                               | 70   |
| Barium 9 (or 10)-p-hydroxyphenyl stearate                    | 0.3                                                                       | 0.2  | 0.5 |      |                       |                                                                | —2   | —2   | —2.8 |    |     |     |                               | >56  |
| Strontium 9 (or 10)-p-hydroxyphenyl stearate                 | 0.2                                                                       | 0.1  | 0.8 | 13.3 |                       |                                                                | 0.1  | —6.2 | —5.8 | 44 |     |     |                               | 81   |
| 240<br>at<br>175° C.                                         |                                                                           |      |     |      |                       |                                                                |      |      |      |    |     |     |                               |      |
| None                                                         | 3.8                                                                       |      |     |      |                       |                                                                | 7    |      |      |    |     |     |                               | 4    |
| 9(or 10)-(2,3-dihydroxyphenyl)stearic acid                   | 2.1                                                                       | 13.5 |     |      |                       |                                                                | 7.6  | 62   |      |    |     |     |                               | 26   |
| 9,12-Bis(4-hydroxyphenyl)stearic acid                        | 0.3                                                                       | 17.5 |     |      |                       |                                                                | 1.8  | 59   |      |    |     |     |                               | 33   |
| Barium 9(or 10)-p-hydroxyphenyl stearate                     | 2.3                                                                       | 12.5 |     |      |                       |                                                                | 5    | 16.5 |      |    |     |     |                               | 28   |

<sup>1</sup> Two percent of the inhibitor in solution unless otherwise indicated.

<sup>2</sup> Determined in accordance with ASTM D664-54.

<sup>3</sup> Determined in accordance with ASTM D445-53T.

atmosphere, excess oxygen pressure was bled off so that 0.1 to 0.5 cm. of pressure remained. Oxygen consumption was calculated as moles of oxygen per mole of compound.

The inhibitor-generating long-chain fatty acids (and salts) of our invention will be hydroxyarylstearyl acids wherein the aryl group is attached to the long acid chain, at various points, through a tertiary carbon. Examples of the type of structures involved are given below:



where  $n+n'=15$   
R=iso-Propyl  
R'=CH<sub>3</sub>



where  $n+n'=15$



where  $n+n'=12$



where  $n+n'=15$   
X=Calcium, Strontium  
or Barium

The above have been found to be compounds effective in inhibiting both oxidation and rust when used in instrument lubricant compositions. The long hydrocarbon chain terminated by the strongly polar acid (or salt) group, adheres to the metal to be lubricated to form a monomolecular layer which prevents rust formation. In addition, hydroxyarylstearyl acids (or salts) are effective as antioxidants because of formation of an inhibitor via autoxidation at the tertiary carbon atom.

In order to determine oxidation stability of the generic group of compounds above-mentioned at different temperatures a dynamic test was employed which is similar to that described in the Federal Specification for "Lubricants, Liquid Fuels, and Related Products; Methods of Inspection, Sampling, and Testing" VV-L-791e, May 21, 1953, Method 5308.3 entitled "Corrosiveness and Oxidation Stability of Light Oils." Two weight percent solutions of the additive compounds in bis(2-ethylhexyl) sebacate, a typical diester lubricant, were oxidized at 120°, 150°, and 175° C. in the presence of copper and steel catalyst strips (1.750 x 0.735 x 0.025 inches). Samples of 10 ml. were withdrawn periodically for viscosity and neutralization number determinations, and the test was continued

The general effectiveness of a particular additive as an antioxidant may rapidly be determined from Table II above by noting the duration of the induction period. That is, the longer the induction period, generally, the more effective the antioxidant. Although all of the hydroxyarylstearyl acids were effective to some extent as antioxidants, excellent results were obtained through the use of 9 (or 10)-(2,3-dihydroxyphenyl) stearic; 9,12-bis (4-hydroxyphenyl) stearic acids; and the alkaline earth salts of 9 (or 10)-p-hydroxyphenylstearic acid.

Rust inhibition data were obtained with the use of a cyclic humidity cabinet wherein test specimens were continuously exposed to alternating cycles of 4 hours at 43.3° C. and 80% relative humidity, followed by 4 hours at 54.4° C. and 95% relative humidity. These conditions are considered severe and give rise to one period of controlled condensation during each 8-hour cycle. Rust inhibition results are presented in Table III below:

TABLE III  
Humidity Cabinet Rust Test Data<sup>1</sup>

| Additive:                                                    | Hours to failure |
|--------------------------------------------------------------|------------------|
| None                                                         | 24               |
| Oleic acid                                                   | 84               |
| Linoleic acid                                                | 72               |
| 9 (or 10)-(2-hydroxy-5-tert-butylphenyl)stearic acid         | 96               |
| 9 (or 10)-(2,3-dihydroxyphenyl)stearic acid                  | 132              |
| 9 (or 10)-(2-hydroxy-3-isopropyl-6-methylphenyl)stearic acid | 96               |
| 9,12-bis(4-hydroxyphenyl)stearic acid                        | 128              |
| Calcium 9 (or 10)-p-hydroxyphenyl stearate                   | 162              |
| Barium 9 (or 10)-p-hydroxyphenyl stearate                    | 186              |
| Strontium 9 (or 10)-p-hydroxyphenyl stearate                 | 132              |

<sup>1</sup> Bis (2-ethylhexyl) sebacate containing 2% of the additive.

From the data presented above, it can be seen that most of the compounds exhibit protection against rust. Since 9 (or 10)-2,3-dihydroxyphenyl stearic; 9,12-bis(4-hydroxyphenyl)stearic acids; and the alkaline earth salts of 9 (or 10)-p-hydroxyphenylstearic acid provide better protection than the more highly substituted compounds, it would appear that the bulky alkyl groups may prevent close alignment of the molecules in the absorbed monolayer or decrease the lateral attractions (Van der Waals forces).

Our combination oxidation and rust inhibitor compounds were prepared as described below, using 9 (or 10)-p-hydroxyphenylstearic acid, and barium 9 (or 10)-p-hydroxyphenyl stearate as examples.

Isomeric arylstearic acids: The 9 (or 10)-arylstearic acids were prepared by the Friedel-Crafts condensation of oleic acid with phenols in the presence of equimolar quantities of anhydrous aluminum chloride. Phenol (7 parts) was mixed with 99% purity oleic acid (1 part) and anhydrous aluminum chloride (1.3 parts) was gradually added with stirring. After the vigorous reaction had subsided, the mixture was heated to 80° C. for 6-8 hours or until the evolution of HCl fumes ceased. The reaction mixture was poured into 20% hydrochloric acid and the organic layer extracted with ethyl ether. The ether extract was washed with water until acid-free and dried over anhydrous Na<sub>2</sub>SO<sub>4</sub>. After filtration, the ether was removed by distillation at atmosphere pressure. Excess phenol was then removed by distillation, in vacuo, until the pot temperature of 150° C. at 1 mm. was obtained. The residue, on distillation from a short-path molecular still at 5-10 microns pressure, yielded 9 (or 10)-p-hydroxyphenylstearic acid. The 9,12-diarylstearic acid was prepared in a similar manner by reaction of linoleic acid with phenol.

The alkaline earth salts of 9 (or 10)-p-hydroxyphenylstearic acid were prepared by conversion of the sodium salt. To a benzene solution of the sodium salt (2 parts) prepared from the free acid and NaOH in a 1:1 ratio was added, dropwise, with stirring, aqueous barium chloride (1 part). The reaction mixture was refluxed for one-half hour, cooled, and poured into a separatory funnel. The product was washed free of chloride and then transferred to a clean flask and the remaining water was removed as

an azeotrope with benzene. Approximately one-half of the benzene was distilled, in vacuo, in a nitrogen atmosphere and then bis(2-ethylhexyl) sebacate was added and the distillation continued until all the benzene was removed. The final product was a concentrated solution (about 20%) of barium 9 (or 10)-p-hydroxyphenyl stearate in bis(2-ethylhexyl) sebacate. The amount of salt was calculated from sulfated ash determinations and the final solution was found to contain less than 0.05% free acid.

10 We claim:

1. A lubricant additive characterized by good oxidative-  
ly autoinhibitive and rust-inhibitive properties, said additive consisting of 9,12-bis(4-hydroxyphenyl) stearic acid.

15

#### References Cited

##### UNITED STATES PATENTS

3,468,920 9/1969 Larimer et al. ----- 260—407

20

##### OTHER REFERENCES

Snead et al.: I & EC Product Research and Development, vol. 5, No. 3, September 1966, pp. 222-225.

25 LEWIS GOTTS, Primary Examiner

E. G. LOVE, Assistant Examiner

U.S. Cl. X.R.

252—57, 393, 404